

## UNITED STATES PATENT OFFICE

FRIEDRICH POSPIECH, OF DRESDEN, GERMANY, ASSIGNOR TO CHEMISCHE FABRIK  
POTT & CO., OF DRESDEN, GERMANY

## METHOD OF ACCELERATING AND IMPROVING TANNING PROCESSES

No Drawing. Application filed August 26, 1927, Serial No. 215,761, and in Germany August 21, 1926.

The hitherto employed tanning processes in which vegetable tanning principles are used are in general, very imperfect, because a very long time is needed for carrying out such processes and the coloring of leather produced in the known tanning processes is not always satisfactory. Normally, the tanning of upper leather, which has been preliminarily tanned in the usual ooze of  $1\frac{1}{2}$ – $2\frac{1}{2}$ ° 10 Bé. and has been finished in an ooze of 6° Bé., lasts for at least 12 to 16 days. Several proposals have been made for shortening the duration of the process but the quick-tanning methods hitherto proposed will not however 15 give entirely satisfactory results, because the grains are tanned before the inner parts of the unhairied hides are tanned, whereby the grains are damaged and the surface of the leather assumes an unattractive look.

20 According to one quick-tanning method, the hides are treated in tanning liquors, which have been enriched by means of non-tanning substances (tannin, gallic acid, resorcin and the like) and are thereupon 25 brought into strong tanning liquors, which are supposed to effect a thorough tanning of the hides in a short time.

According to another proposal, the hides, that is, the grained parts of the same are 30 treated with inorganic salts adapted to make the grains non-sensitive to the astringent effects of strong tanning liquors (alumen, Glaubers salt, kitchen salt, bitter salt in combination with bichromate, boric acid, oxalic acid, chloride of calcium, hydrochloric aniline).

The first of the processes mentioned is expensive, and on account of the sensitiveness of the employed substances to iron, is not to 40 be depended upon. Further the tanning lasts for at least 3 to 4 days, because the liquor at the first stages of treatment must not be stronger than 3 to  $3\frac{1}{2}$ ° Bé. in order that the grains are not damaged.

45 The initial treatment with inorganic salts, in accordance with the second of the above mentioned proposals, is always risky, because conversion with the vegetable tanning agents may take place, whereby the coloring properties, the softness, the flexibility and the touch

of the grains are affected in an unfavorable manner. When chromium salts and aluminum salts are used also the character of the leather is changed, so that a product is obtained, which resembles the so-called semi-chrome-leather. 55

I have now found, that the above mentioned drawbacks are avoided and the duration of the tanning process is markedly shortened when substances are added to the 60 tanning liquors which will reduce the surface tension in aqueous solutions. Such substances are for instance, aromatic sulphonic acids and salts of the same. The products obtained by my new process are of the same 65 quality as the leather obtained by the former processes and are with respect to the coloring qualities superior to the leather hitherto obtained. 70

Especially suited for the purpose are sulphonic acids which are obtained by condensing naphthalene or ring substitution products of naphthalene, or the corresponding sulphonic acids, in the presence of condensation or oxidation agents with alcohols of the aliphatic series, having more than two carbon atoms. 75

Such substances may, for instance, be produced by converting one molecule of naphthalene into a mixture of alpha and beta sulphonic acids and bringing the same into reaction with 2.1 molecules of isopropyl-alcohol and 2.1 molecules of concentrated sulphuric acid at temperatures below 100° C. and in the presence of a large quantity of concentrated sulphuric acid. The sodium salt, obtained in the usual way by treating with lime water and boiling the thus obtained sulphonic acid of the condensation product of naphthalene and iso-propyl alcohol, forms 85 directly a suitable addition for the tanning process to be described.

Instead of naphthalene, other polynuclear aromatic hydrocarbons and substitution products of such substances, as for instance, 90 halogen or hydroxy substituted compounds, may be used. Instead of iso-propyl alcohol also higher alcohols especially such of the secondary series may be employed. Further aliphatic and cyclic olefines, such as tetra- 100

hydrobenzol dissolved in concentrated sulphuric acid, are well suited for the purpose in question. The condensation products are amorphous substances which very easily dissolve in water and which as free acids and also as alkali salts possess a considerable moistening and frothing ability.

*Example 1*

10 100 kg. of unhaired hides, which are designed for tanned upper leather and which, therefore, have been accordingly treated in the lime pit, are unlimed and eventually soaked. These hides are not as usual brought 15 into a diluted color solution (tanning liquor of 0.5 to 1.5° Bé.) but are treated with a solution of 2 kg. of one of the above named substances in 300 liters of water for 3 to 4 hours, whereupon the hides are directly brought in 20 to a tanning liquor of 4 to 6° Bé., which is sufficiently strong to effect the final tanning. The tanning may be performed in drums or vats. As a tanning agent any vegetable extract or mixture of different extracts may be 25 used. The entire tanning process lasts for 24 to 36 hours.

*Example 2*

30 100 kg. of unhaired hides, which are designed for bottom leather and have been accordingly treated, are unlimed as completely as possible by means of an organic acid (lactic acid, formic-acid, butyric acid or the like). Thereupon 2 kg. of one of the above named 35 substances are added to the same bath (or to a fresh bath) and are allowed to act upon the hides. For this purpose small amounts of organic acids may be added anew in order that the unhaired hides may be raised sufficiently. After 3 to 4 hours the hides can be 40 put into the tanning bath. Any vegetable extract may be used. The extract is chosen in accordance with the purpose for which the finished product is intended to be used.

*Example 3*

45 The treatment of unhaired hides can also be performed in a weak tanning liquor to which 2 kg. of one of the above named substances are added for each 100 kg. of hides.

50 I claim:

1. A method of accelerating and improving the tanning processes when working with vegetable tanning agents, which comprises adding to the tanning liquor, condensation products of naphthalene sulfonic acids and alcohols of the alipathic series having more than two carbon atoms in the presence of condensation mediums.
2. A method of accelerating and improving the tanning processes when working with vegetable tanning agents, which comprises adding to the tanning liquor sulphonic acids of propylated naphthalene.

65 FRIEDRICH POSPIECH.